

## UNITED STATES PATENT OFFICE

WILLIAM C. CALVERT, OF AKRON, OHIO, ASSIGNOR TO THE GOODYEAR TIRE & RUBBER COMPANY, OF AKRON, OHIO, A CORPORATION OF OHIO

## GAS CELL FABRIC

No Drawing.

Application filed April 8, 1930. Serial No. 442,696.

This invention relates to coated fabrics and has particular relation to fabrics of the kind employed in the construction of gas cells for lighter-than-aircraft. It is not, however, limited in its usefulness to such gas cells, for it may be used wherever a fabric is desired possessing the properties characterizing the herein described material.

One object of the invention is to provide a fabric which offers exceptionally high resistance to permeation by hydrogen and helium.

Another object of the invention is to provide a fabric which is exceptionally light of weight, durable and flexible.

A third object is to provide a fabric having the above designated characteristics, the units of which may be spliced together by means of moisture-proof rubber cements.

Other objects will be apparent as the description of the invention proceeds.

For convenience, the invention will be described hereinafter as applied to lighter-than-aircraft, but it will be understood that it is in fact not limited thereto, being capable of being put to many other uses.

The gas cells of lighter-than-aircraft are usually constructed of light, strong, closely woven cotton textile material which is coated with a continuous film of a highly impervious substance designed to prevent unduly rapid diffusion of the imprisoned gases. Although many materials have heretofore been employed for coating these fabrics, only two materials, rubber and gold beater's skin, have heretofore been considered to possess the requisite properties for extensive commercial use.

Rubber is abundant and relatively cheap to obtain and may also be applied to the fabric by mechanical means with a minimum expenditure of time and labor. It is also impermeable to moisture and units thereof may readily be secured together by means of rubber cements which are also not affected

by moisture. In these respects, rubber is almost an ideal material. However, it is also subject to serious objections. For example, the permeability thereof is comparatively high and accordingly, it is necessary to employ coating films of excessive thickness and weight in order to obtain sufficient resistance to the escape of the inflating gases. Furthermore, when it is spread in relatively thin films upon ordinary fabrics, it is subject to relatively rapid decay. Within a comparatively short time, it is likely to crack and check, thus leaving openings through which the imprisoned gases may escape.

Gold beater's skin is obtained in the form of relatively small strips or units from the viscera of cattle. It is necessary to subject it to tedious processing in order to obtain it in form suitable for application to fabric. The units thereof are applied to the fabric by means of some convenient cement such as rubber or glue. Since these units are comparatively small in size, much time and labor is necessary in order to spread it upon such extensive surfaces as exist in gas cells of lighter-than-aircraft. However, it is quite tough, flexible and affords very high resistance to permeation by gases. In these respects, it is markedly different from the rubber coatings. In the construction of gas cells for rigid craft of the Zeppelin type, where it is necessary to imprison great quantities of gases over long periods of time, these advantages have been found to outweigh the disadvantages. Therefore, it has found extensive application in this type of aircraft even though the expense of application is great.

Heretofore, much time and effort has been expended in an effort to develop a synthetic material having the lightness and durability of gold beater's skin which may be obtained and applied with an expenditure of effort more nearly approximating that of rubber. Although numerous compositions such as nitrocellulose and other esters of cellulose

have been suggested, none of them has been found to be entirely practicable. For example, some have been unduly permeable to inflating gases. As a specific example of this type of material, mention may be made of nitrocellulose which, although apparently extremely dense and impermeable, is found by actual experience to permit the loss of fifteen liters of inflating gas per square meter of fabric. Furthermore, most of these compositions are objectionable because it is difficult by ordinary means to secure units thereof together by means of the common cements. Various other objectionable features such as inflexibility and lack of durability have also been encountered in connection with some of the materials heretofore proposed.

The present invention consists in the provision of a composition consisting of gelatin, latex and a softening ingredient such as polyglycerol applied to the fabric in such manner that substantially all of the objections heretofore encountered in connection with gold beater's skin or rubber coatings for gas cell fabric are substantially overcome while the advantages of both are retained.

In practicing the invention, a suitable gas cell fabric is preferably spread with a very thin light coating of rubber weighing approximately 0.8 ounces per square yard. This material may be spread upon a single side of the fabric, but it is preferable to apply it to both sides in order to reduce the tendency of the fabric to curve upon application of solvents for purpose of seaming the units of fabric together. This coating is then succeeded by a second coating of self curing rubber cement which may have the following formula:

|                                   | Per cent<br>by weight |
|-----------------------------------|-----------------------|
| Rubber                            | 4.9                   |
| Zinc oxide                        | 0.265                 |
| Sulfur                            | 0.078                 |
| 45 Captax (mercaptobenzothiazole) | 0.090                 |
| Diethylamine                      | 0.047                 |
| Benzol                            | 34.840                |
| Naphtha                           | 59.780                |

The third coating consists of a film of latex which may vary in composition but which preferably should contain approximately 67.5 percent of rubber. Additional coatings comprising mixtures of gelatin, latex and polyglycerol are then applied to the rubber base. In these coatings, the first plies are composed of relatively large percentages of latex and correspondingly small proportions of gelatin. However, the ratio of gelatin to latex is gradually increased in succeeding plies until eventually a number of plies of pure and nearly pure gelatin or polyglycerol are applied. The gelatin-polyglycerol coatings are succeeded by a number of coatings of a gelatin, polyglycerol and latex mixture which readily adhere to the gelatin surface.

Finally, the fabric is coated with a plurality of films of substantially pure latex and, if desired, is then dressed with an outer coating of a suitable varnish, lacquer or rubber coating. Paraffin or similar material may be applied to the latter to increase the water resistance.

In practicing the invention, two solutions termed respectively "A" and "B" are employed. Solution A comprises

|                                      | Grams    |
|--------------------------------------|----------|
| Rubber latex (67.5% rubber)          | 150      |
| Sodium hydroxide (70% concentration) | 7.5      |
| Water                                | 217.5 80 |

The composition of Solution B is as follows:

|              | Grams  |
|--------------|--------|
| Gelatin      | 200 85 |
| Polyglycerol | 450    |
| Water        | 1572   |

The exact order of application and composition of the various coatings may be tabulated as follows:

|                                                                                                                               | Oz. sq. yd. |
|-------------------------------------------------------------------------------------------------------------------------------|-------------|
| Coat #1—Self curing rubber cement (containing sulfur and ultra accelerator e. g. mercaptobenzothiazole salt of diethyl amine) | .05 .05     |
| Coat #2—Solution A                                                                                                            | .10         |
| Coat #3—80 grams Solution A, 120 grams Solution B, 80 grams water                                                             | .07         |
| Coat #4—40 grams Solution A, 240 grams Solution B                                                                             | .05 100     |
| Coats #5-18—Solution B                                                                                                        | 1.00        |
| Coat #19—40 grams Solution A, 240 grams Solution B                                                                            | .05         |
| Coat #20—40 grams Solution A, 240 grams Solution B                                                                            | .05 105     |
| Coat #21—100 grams latex (67.5% rubber content) 93 grams water                                                                | .05         |

It is to be understood that each coating or film of material is permitted to dry before the succeeding coating is spread. It is also essential that the fabric be maintained under tension by suitable means such as stretching frames or other convenient devices in order to insure that it will be smooth and free from wrinkles. When properly prepared, gas cell fabrics of ordinary type, weighing approximately 2.8 ounces per square yard, are found to have a weight of approximately 4.22 ounces per square yard. Such fabrics permit a diffusion of approximately .21 liters of hydrogen per square meter during a period of 24 hours. This loss is comparatively small, in fact, it is probably even less than that permitted by gold beater's skin. The exterior latex coatings also function admirably as foundations for rubber cements which may be employed to bond the various units of fabric together. This is a distinct advantage over most of the substitutes for gold beater's skin

heretofore suggested because the latter cannot be secured by means of such cements. Indeed, in connection with most of these materials, one of the most difficult problems heretofore encountered has been to obtain an adequate seam for the various units.

Although I have described the preferred embodiment of the invention, it will be apparent to those skilled in the art that it is not limited thereto but that various modifications may be made therein without departing from the spirit of the invention or from the scope of the appended claims. It is intended that that the patent shall cover, by suitable expression in the appended claims, whatever features of patentable novelty reside in the invention herein disclosed.

What I claim is:

1. A method of treating balloon fabric which comprises spreading thereon a coating of rubber, spreading latex upon the rubber, then spreading a coating of a mixture of latex and gelatin, adding intermediate coatings of gelatin and polyglycerol, applying a coating consisting of a mixture of gelatin, latex and polyglycerol and finally adding an exterior coating consisting essentially of latex.

2. A method of preparing balloon fabric which comprises coating a light strong closely woven fabric base with a self curing rubber cement, spreading a coating of latex and gelatin upon the cement, adding a coating of a mixture of gelatin and polyglycerol followed by a coating of a mixture of latex gelatin and polyglycerol, and finally applying a coating consisting essentially of latex.

3. A gas cell for lighter-than-aircraft comprising a closely woven cotton fabric base, a film of rubber upon the base, an intermediate film consisting essentially of gelatin and polyglycerol, and an outer ply consisting essentially of rubber.

4. A method of manufacturing coated fabrics which comprises coating a fabric base with rubber, spreading latex upon the rubber, spreading a mixture of latex and gelatin upon the latex, adding an intermediate coating of gelatin and a softener, coating the gelatin with a mixture of latex and gelatin, and finally dressing the latter coating with latex.

5. A gas cell for lighter-than-aircraft comprising a closely woven cotton fabric base, a film of rubber upon the base, an intermediate film consisting of gelatin and polyglycerol, and an outer coating consisting essentially of rubber which is coated with paraffin or similar material.

6. A gas cell construction for lighter-than-aircraft embodying a plurality of units of textile fabric, one of which at the line of union is coated with a layer comprising rubber as its principal ingredient, a layer comprising gelatin and polyglycerol as essential in-

gredients, and an outer layer consisting primarily of rubber, the latter layer being joined to the other unit by means of rubber cement.

7. A gas cell fabric for lighter-than-aircraft comprising a base of light textile material, inner and outer coatings consisting essentially of rubber upon the base, an intermediate coating consisting essentially of gelatin and polyglycerol between the rubber coatings.

8. A gas cell fabric for lighter-than-aircraft comprising a light, closely woven textile material, inner and outer coatings upon the fabric consisting essentially of rubber and an intermediate coating comprising gelatin and polyglycerol between the rubber coatings, the latter being blended in progressively decreasing proportions into the intermediate coatings.

9. A gas cell fabric for lighter-than-aircraft comprising a base of light fabric, inner and outer coatings of rubber upon one side of the base, an intermediate coating comprising polyglycerol, and a medium highly resistant to permeation by hydrogen and helium intermediate the rubber coatings.

10. A gas cell construction comprising a plurality of units of fabric, each unit comprising inner and outer layers of rubber and intermediate layers of a material highly resistant to diffusion gases, the units being joined together by means of rubber cement.

In witness whereof, I have hereunto signed my name. Signed at Akron, in the county of Summit and State of Ohio, U. S. A., this 7th day of April, 1930.

WILLIAM C. CALVERT.

105

110

115

120

125